

G. M. WILLIS.  
PROCESS AND APPARATUS FOR EXTRACTING BITUMEN FROM BITUMEN BEARING ORE,  
APPLICATION FILED MAR. 27, 1907.

918,628.

Patented Apr. 20, 1909.



Witnesses:

Leonard W. Moander  
Fred W. Koch.

Inventor  
George M. Willis  
By Charles A. Brown  
Attorney

## UNITED STATES PATENT OFFICE.

GEORGE M. WILLIS, OF CHICAGO, ILLINOIS.

## PROCESS AND APPARATUS FOR EXTRACTING BITUMEN FROM BITUMEN-BEARING ORE.

No. 918,628.

Specification of Letters Patent. Patented April 20, 1909.

Application filed March 27, 1907. Serial No. 364,821.

*To all whom it may concern:*

Be it known that I, GEORGE M. WILLIS, citizen of the United States, residing at Chicago, in the county of Cook and State of Illinois, have invented a certain new and useful Improvement in Processes and Apparatus for Extracting Bitumen from Bitumen-Bearing Ore, of which the following is a full, clear, concise, and exact description, reference being had to the accompanying drawings, forming a part of this specification.

My invention relates to an improved process for extracting bitumen in its pure state from bitumen bearing sand.

In accordance with my invention the ore or rock is first ground or disintegrated to a suitable degree, say, about twenty meshes to the inch. This powder, which is a mixture of sand and asphalt, is mixed with water in a suitable vessel and heated, the clear sand, being of great specific gravity, dropping to the bottom of the receptacle, and the asphalt and some sand mixing with the water to form a scum which remains more toward the top of the receptacle. The precipitating sand is continuously carried away from the receptacle and the scum is kept agitated by being mixed with air under more or less pressure, this air agitation taking place in another suitable receptacle, and more sand is liberated and settles to the bottom of the second receptacle, whence it may be continuously withdrawn in any suitable manner. The scum leaving the first receptacle has approximately 60% sand and 40% bitumen or asphalt, while the scum after treatment in the second receptacle becomes 70% pure and containing only about 30% sand. The scum from the second receptacle is then passed over the heating surface and suitably heated to about 600 degrees Fahrenheit, the heating surface being inclined and of such length that when the scum leaves the surface it will have been thoroughly dried. The dry substance is collected in a suitable tank or receptacle which is suitably heated from the outside. In this tank the remaining sand in the mixture settles to the bottom of the tank, while the pure asphaltum is lighter and fills the top of the receptacle, whence it may be withdrawn. The residuum in the tank consists in greater part of sand, and this residuum is extracted and re-fed into the first receptacle. The process is a continuous one, the ground ore or rock being continuously

fed to the first receptacle and the residuum from the last settling tank being constantly added to the first receptacle, and pure asphaltum can constantly be drawn off.

Many forms of apparatus can be employed for carrying out my process, and in the accompanying drawing I show one form and arrangement of apparatus which I find is readily adapted to carrying out my invention in a very efficient manner.

In this drawing Figure 1 is a more or less diagrammatic top view of the various parts of the apparatus showing the sequence of operations, and Fig. 2 is a sectional view taken on line 2-2 of Fig. 1.

The ore or rock is first suitably ground and disintegrated and fed as through a hopper 1 to one end of a tank 2, which tank is comparatively long and, say, about two feet deep. This tank connects with a second tank 3 which is offset and to the side of tank 1, as shown, the two tanks being connected by the passageway 4. At the ends of the first tank are rollers 5 and 6 about which passes an endless chain or rabble 7. The shaft 8 of roller 5 may be suitably driven from a motor or engine, and a belt 9 may be used to transmit rotation from shaft 8 to shaft 10 of roller 6. The chain is so arranged that the upper part between the rollers passes along in engagement with the floor of the tank 2, the direction of travel being as indicated by the arrows. This tank 2 is also nearly filled with water and below the tank heat is employed, as by means of hydro-carbon burners 11. The water is thus heated to boiling and the mixture of asphaltum and sand is also thoroughly heated and more or less agitated by the boiling water. A considerable quantity of sand is liberated and falls to the bottom of the tank, and the links of the chain or rabble are so formed that as the chain travels the sand will be carried therewith and expelled from the chain as it passes over the roller 6. A mixture of the asphaltum, sand and water forms a sort of scum at the top of the tank, and this scum, owing to the movement of the chain, is carried and deflected into the passageway 4 and thence into the second tank, which also contains water and is heated by other burners. Air under suitable pressure is led into the mass through twyvers 12 which enter the sides of the tank 3 just below the surface of the liquid in the tank and terminate flush

65

70

75

80

85

90

95

100

105

110

with the inside of the same and the mixture of asphaltum, water and sand is thoroughly agitated, partly by the results of boiling and more so by the incoming air, and more sand is liberated. The liberation of sand in the first tank is such that the scum contains about 40% asphaltum and 60% sand, while after treatment in the second tank the amount of sand will have been reduced so 10 that the scum will contain about 70% asphaltum and 30% of sand. The sand liberated upon treatment in the second tank settles to the bottom of the tank and may be removed in any suitable manner, as through traps or 15 by means of a traveling chain or conveyor similar to that passing through the first tank. After treatment in the two tanks just described, the scum in tank 3 is dried and for this purpose is caused to pass over a heating 20 surface, which may be an inclined chute 13, as shown, this chute leading from the end of tank 3 and into a tank or receptacle 14. The scum is carried from tank 3 to the chute by means of a paddle wheel 15, as shown, 25 this paddle wheel being shown as mounted over the right end of the tank 3 and on a shaft 16 which may be driven by a belt 17 connected with shaft 10. The travel of the scum is maintained by means of the chain 30 running through the first tank and by means of the paddle wheel, which paddle wheel scoops the scum from tank 3 on to the chute. This chute is heated to, say, about 600 degrees Fahrenheit throughout its entire length 35 and before the scum leaves the chute it is thoroughly dried of all moisture. Tank 14 is also heated and in this tank pure asphaltum is finally obtained. After being thus highly heated upon its passage over the inclined 40 chute, then when it reaches tank 14, the lighter clear liquid asphaltum will remain at the top of the tank, while the heavier substance, which still retains sand, will settle to the bottom. The clear asphaltum is then 45 drawn from the tank 14, while the residuum, which contains a great amount of sand, is re-treated by being re-fed to the first tank with fresh ore.

By means of my process I am enabled to 50 break up in stages the great affinity which asphaltum, or like bituminous substances, has for sand, by first causing mechanical disintegration thereof, and then continually heating it and keeping it thoroughly agitated 55 during such heating.

I do not wish to be limited to the precise apparatus and mechanism shown for carrying out my process, nor to the exact sequence of operations which I have described, as 60 changes may readily be made without departing from the scope of my invention.

I desire to cover the following method claims by Letters Patent:

1. The process of extracting asphaltum 65 from asphaltum-bearing ore, which consists

in grinding the ore, heating the ground ore in water to cause release of some of the sand and foreign matter, removing the sand and foreign matter upon release thereof, further heating the residue in water, introducing air 70 under pressure into the floating mass to cause agitation of the mixture whereby more sand is liberated, then drying the residue, then filling it into settling tanks in which the remaining sand and foreign matter is precipitated and from which the clear asphaltum 75 can be drawn off.

2. The process of extracting bitumen from bitumen-bearing ore which consists in grinding the ore to a sand, heating the sand in water and causing agitation of the resulting floating mass to release the sand, removing the precipitated sand, then causing the residue to flow in a thin stream, and heating it 80 to drive the moisture therefrom. 85

3. The process of extracting bitumen from bitumen-bearing ore which consists in grinding the ore, heating the ground material in water to cause precipitation of some of the sand, further heating the residue in water and at the same time blowing air into the floating mass to cause further agitation thereof and to assist in the liberation of more sand, then causing the residue to flow in a thin stream and to be heated to drive the 90 moisture therefrom, and then heating the dried residue to cause precipitation of the remaining sand. 95

4. The process of extracting bitumen from bitumen bearing ore which consists in 100 grinding the ore to a finely divided condition, in mixing the particles thus produced with water in a first treating tank, in heating the mixture in the first tank, in transferring the floating bitumen particles to a second 105 tank, in agitating the floating mass in the second tank, and in then heating the remaining bitumen particles and allowing the remaining impurities to settle.

5. The process of extracting bitumen 110 from bitumen bearing ore which consists in grinding the ore to a finely divided condition, in mixing the particles thus produced with water, in heating and agitating the mixture to produce a floating mass of the bitumen particles, in removing the floating mass from the influence of such heating and agitating action, in there agitating the floating mass, and in then heating the bitumen particles and allowing the remaining impurities 115 120 to settle. 125

6. As a means for separating bitumen from pulverized bitumen ore, means for heating and agitating the pulverized ore with water to produce a floating mass of bitumen particles on the water, means for removing the floating mass from the location of such heating action, means for agitating the floating mass without agitation of the water beneath it, and means for drying and purifying 130

the remaining mass of floating bitumen particles.

7. As a means for separating bitumen from pulverized bitumen ore, means for 5 heating and agitating the pulverized ore with water to produce a floating mass of bitumen particles on the water, means for removing the floating mass from the location of such heating action, means for agitating 10 the floating mass without agitation of the water beneath it, and means for removing the moisture from the mass of bitumen particles.

8. As a means for separating bitumen 15 from pulverized bitumen ore, means for heating and agitating the pulverized ore with water to produce a floating mass of bitumen particles on the water, means for removing the floating mass from the location of such 20 heating action, means for agitating the floating mass without agitation of the water beneath it, means for removing the moisture from the mass of bitumen particles, and means for removing remaining 25 impurities from the dried bitumen.

9. As a means for separating bitumen from pulverized bitumen ore, means for delivering the pulverized ore to a first treating pan, means for heating and agitating the 30 pulverized ore with water in such pan to produce a floating mass of bitumen particles on the water, means for removing the floating mass to a second pan, means for agitating the 35 floating mass in the second pan without agitation of the water beneath it, and means for drying and purifying the remaining mass of floating bitumen particles.

10. As a means for separating bitumen from pulverized bitumen ore, means for 40 delivering the pulverized ore to a first treating pan, means for heating and agitating the pulverized ore with water in such pan to produce a floating mass of bitumen particles on the water, means for removing the 45 floating mass to a second pan, means for agitating the floating mass in the second pan without agitation of the water beneath it, means for removing the moisture from the mass of bitumen particles, and means for 50 removing remaining impurities from the dried bitumen.

11. As a means for separating bitumen from bitumen bearing ore, a treating pan, means for supplying pulverized ore to be 55 treated to such pan, means for heating and agitating the pulverized ore with water to produce a floating mass of bitumen particles, means for removing the floating mass from the location of such heating action, 60 means for agitating the floating mass without agitating the water beneath it, means for removing the bitumen particles to a drying pan, and means for removing remaining impurities from the dried bitumen.

65 12. As a means for separating bitumen

from bitumen bearing ore, a first treating pan, means for supplying pulverized ore to be treated and water to such pan, means for heating and agitating such pan to produce a floating mass of bitumen particles, a 70 second treating pan, means for transferring the floating mass thereto, means for agitating the floating mass in the second pan without agitating the water beneath it, a heated drying pan, means for transferring 75 the bitumen particles to such drying pan, and means for removing remaining impurities from the dried bitumen.

13. As a means for separating bitumen from pulverized ore consisting principally 80 of bitumen, sand and silt, is finely divided and intermingled condition, means for delivering the pulverized ore to a treating pan, means for heating and agitating the pulverized ore with water in such pan to produce 85 a floating mass of bitumen particles on the water and to precipitate a part of the sand from the pulverized ore, means for removing the floating mass from the location of such heating action, means for agitating the floating mass without agitation of the water beneath it to effect the precipitation of the sand remaining in the floating mass, means for removing the moisture from the mass of bitumen 90 particles, and means for removing the silt from the dried bitumen.

14. As a means for separating bitumen from pulverized ore consisting principally 100 of bitumen, sand and silt, in finely divided and intermingled condition, means for delivering the pulverized ore to a first treating pan, means for heating and agitating the pulverized ore with water in such pan to produce a floating mass of bitumen particles on the water and to precipitate a portion 105 of the sand contained in such pulverized ore, means for transferring the floating mass to a second treating pan, means for agitating the floating mass in such second pan without agitation of the water beneath it to effect the precipitation of the sand remaining in the floating mass, means for removing the moisture from the mass of bitumen particles, and means for removing 110 the silt from the dried bitumen.

15. As a means for separating bitumen from pulverized bitumen bearing ore, means for delivering the pulverized ore into a first 120 pan containing water, means for heating the pan and its contents and thereby separating and precipitating a portion of the sand contained therein, means for transferring the bitumen particles and remaining impurities to a second pan, means for agitating the mixture in such second pan, 125 means for heating such second pan and its contents, such agitation and heating serving to precipitate more of the sand from the mixture, means for removing the bitumen 130

4  
particles and remaining impurities to an inclined pan, means for heating such inclined pan to drive off the water mixed with the bitumen and to render it fluid, and a settling tank for receiving the fluid bitumen from the inclined pan.

16. As a means for separating bitumen from pulverized bitumen bearing ore, means for delivering the pulverized ore into a first pan containing water, means for heating the pan and its contents and thereby separating and precipitating a portion of the sand contained therein, means for transferring the bitumen particles and remaining impurities to a second pan, means for agitating the mixture in such second pan, means for

heating such second pan and its contents, such agitation and heating serving to precipitate more of the sand from the mixture, means for removing the bitumen particles 20 and remaining impurities to a third pan, means for heating such third pan to drive off the water mixed with the bitumen and to render it fluid, and a settling tank for receiving the fluid bitumen.

In witness whereof, I hereunto subscribe my name this 25th day of March A. D., 1907.

GEORGE M. WILLIS.

Witnesses:

CHARLES J. SCHMIDT,  
GEORGE E. HIGHAM.